

## UNITED STATES PATENT OFFICE

CHARLES SAMUEL HOLLANDER, OF PHILADELPHIA, AND EDWARD LESLIE HELWIG, OF  
BRISTOL, PENNSYLVANIA

## REACTIVE PACKING FOR METALLURGICAL REFRactories

No Drawing.

Application filed February 6, 1929. Serial No. 338,021.

In the operation of electric furnaces a crack in the refractory wall is always a source of danger. This is especially true if the charge consists of molten or boiling metal as the flow 5 of material through a refractory break would immediately endanger any resistors or inductors used to produce the heating effect. It would consequently be a decided advancement in the state of the art to be able to seal up such 10 cracks as they are formed and thus prevent the charge from escaping. This we propose to do by backing the crucible or retort with a layer of granular, powdered or sintered material containing a constituent which will, at 15 the temperature encountered, react with the material of the charge to form a product which is solid or plastic at the prevailing temperature. In case of a crack then the molten or vaporized charge will immediately encounter this reactive material and the products of 20 the reaction will block its flow.

We are aware that, in the past, crucibles and retorts have been coated on the outside with materials to prevent the flames or gases 25 of a combustion furnace from attacking the body of the refractory. Graphite crucibles, for instance, have been given a siliceous outer coating for this purpose. However this is totally different from the purpose of our in- 30 vention.

It has also been general practice in the past to back the crucibles in induction furnaces with a granular refractory for the purpose of supporting the crucibles. In the event of a 35 break, this would mechanically absorb a certain amount of the charge in its pore space but would not necessarily react with it to form a repair. Since it does not react, there is a great danger of the unreacted charge chemically at- 40 tacking the coils or short circuiting them.

*Example 1.*—A clay-graphite crucible is sawed in half and the saw cut scarred with a file. This is to imitate a cracked crucible. It is placed inside a larger clay-graphite crucible 45 and the space between them is packed tightly with a mixture of four parts finely ground silica and one part monobasic sodium phosphate. The inner crucible is filled with metallic zinc. The whole assembly is placed 50 in an electric resistance furnace and heated

until the zinc boils vigorously. It is then cooled, taken apart and examined. It is found that the zinc has filled the file marks in the saw cut and has begun to leak through into the packing. No metallic zinc is found in 55 the packing however. Instead, a half inch, hemispherical zone of sintered material is found at the end of each file mark which shows the extent to which the reaction has penetrated. The crack is effectively sealed 60 and the charge retained inside the broken crucible.

The experiment is repeated, substituting silica powder alone for the mixture described above. At the end of the experiment the bulk 65 of the charge is found in the bottom of the outer crucible and zinc is found disseminated throughout the packing. No reaction occurs in this case while in the former experiment a true chemical reaction occurs between the 70 packing and the charge.

*Example 2.*—A clay-graphite retort containing zinc is surrounded by an inductor coil. The space between the crucible and the coil is tightly packed with a mixture of one part 75 acid sodium phosphate and four parts finely ground silica. The zinc is brought to boiling by power applied to the inductor coil. In the event of a break in the crucible, the zinc vapor or molten zinc, as it emerges from the retort, 80 immediately reacts with the constituents of the packing forming a plastic material which prevents a further flow of metal from the break.

*Example 3.*—The clay-graphite crucible 85 used in Example 1 is charged with iron sulphide and it is surrounded with a tightly packed layer of a mixture of three parts silica powder and one part sodium carbonate. It is heated well above the melting point of the iron sulphide, then cooled and examined. The charge has been retained inside the broken crucible and the cracks effectively sealed. 90

These examples are merely given by way of 95 illustration and should not be taken as limiting us in the application of this principle. It is only limited to the use of such materials as will react with the charge at the prevailing temperature and is applicable to all types of 100

furnaces where a packing may be used to surround the charge container.

We claim as our invention—

1. The process of blocking egress of a charge in case of a refractory failure of a crucible or retort by surrounding the crucible or retort with a packing which will react chemically with the contents to form a plastic mass at the prevailing temperature.
- 10 2. The process of blocking egress of a charge in case of a refractory failure of a crucible or retort by surrounding the crucible or retort with a packing composed of a mixture of silica and an alkali salt which will react chemically with the contents to form a plastic mass at the prevailing temperature.

Dr. CHARLES SAMUEL HOLLANDER.

EDWARD LESLIE HELWIG.